

# UNITED STATES PATENT OFFICE.

JAMES H. MADDY, OF NEW YORK, N. Y., AND BRUNO H. SCHUBERT, OF WEEHAWKEN, NEW JERSEY, ASSIGNORS TO THE IOHMAN COMPANY, OF NEW YORK, N. Y., A CORPORATION OF NEW YORK.

## FLUX FOR COATING METAL BATHS.

1,189,373.

Specification of Letters Patent.

Patented July 4, 1916.

No Drawing. Application filed February 2, 1915, Serial No. 5,643. Renewed December 2, 1915. Serial No. 64,776.

To all whom it may concern:

Be it known that we, JAMES H. MADDY, residing at 610 West One Hundred and Sixteenth street, New York, county of New York, and State of New York, and BRUNO H. SCHUBERT, residing at 224 Jane street, Weehawken, county of Hudson, and State of New Jersey, both citizens of the United States, have invented certain new and useful Improvements in Fluxes for Coating Metal Baths, fully described and represented in the following specification and the accompanying drawings, forming a part of the same.

15 The object of this invention is to facilitate the formation of a coating upon metallic articles by immersing in a molten bath, and the invention relates to the use of a flux of particular character, which is especially 20 useful and desirable in connection with a molten bath composed of lead or other metal.

The flux and processes herein described can be used with baths of molten zinc and various alloys which are fusible near the 25 temperature of melted lead.

The invention includes a particular process of forming a flux of zinc chlorid with an excess of ammonium chlorid upon the surface of a molten bath, and also the process of 30 coating ferrous articles in the molten bath by the joint use of such flux and the treating of the ferrous articles with a salt of mercury before its immersion in the bath.

Ammonium chlorid, on account of its 35 cheapness, has heretofore been used as a flux mixed with bran, flour, or other binders, with the purpose of protecting the surface of the molten metal from oxidation; but such a flux produces objectionable 40 charred or inert substances upon the bath, and produces no beneficial effect upon the surface of the article that is dipped into the metal; whereas the compound flux herein described has a material cleaning effect 45 upon the metal article, so that if slight defects in cleaning exist, the flux removes any oxid upon the surface of the article and the molten metal is thus enabled to adhere perfectly thereto and coats the article thoroughly without permitting the formation of any pin-holes.

Articles coated with lead, zinc, or alloys of lead and zinc with tin, and especially

articles of iron or steel, may thus be furnished with an integral coating which protects them from rust and maintains such protection for a long period.

When new metal is placed in the pot to be melted it often carries oxids, which tend to attack the surface of the articles immersed therein; but with the flux described herein, the surface of the article is effectively protected from oxidation, and the molten metal is thus enabled to coat the article more perfectly.

The present invention is especially useful in the coating of ferrous articles which have been previously treated with salt of mercury to promote the adhesion of the molten metal thereto, as the flux operates to prevent oxidation of the mercury which is formed upon the surface of the article by deposition from the salt, when heated by immersion in the molten bath.

The efficiency of the compound flux is due 75 largely to the presence of the zinc chlorid, which prevents the formation of oxids and assists to clean the surface of the article as it is immersed in the molten bath; but zinc chlorid is ten times as costly as ammonium 80 chlorid and is much more volatile, so that it is soon dissipated if used alone as a flux.

A great saving is secured by using ammonium chlorid in the flux, in much greater proportion than the zinc chlorid, as it prevents the zinc chlorid from vaporizing and 85 enormously reduces the cost of the flux.

The preferred method of preparing and using the flux is as follows: A flux stock solution is prepared of zinc chlorid, either 90 alone or saturated with an excess of ammonium chlorid dissolved therein. This solution is poured upon the metal in the melting pot either when cold or when melted and when the metal is hot the flux is evaporated 95 into a thick black liquor cohering together in a mass, covering not more than one-half the surface of the molten metal. That is, only sufficient of the solution is poured into the pot to form such a partial covering for 100 the molten metal. To this black mass containing zinc chlorid, is then added sufficient commercial ammonium chlorid to form a black or thick liquid covering the entire surface of the metal in the pot to a depth of 105 from one-eighth to one-half of an inch.

When this coating becomes black and spreads over the entire surface of the melted metal, the flux is completed, and will last for a week or ten days in constant use. This compound flux is formed more quickly in the pot and spreads more evenly over the surface than a flux formed wholly of ammonium chlorid with such a binder as bran, and can be applied to the molten metal with 10 more ease, and more certainty of its subsequent operation than bran-ammonium flux.

The capacity of the compound flux to spread freely over the molten metal is especially useful in application to a lead bath 15 or one composed chiefly of lead, as the lead for some reason tends to cake mere ammonium chlorid which caking exposes portions of the molten bath to oxidation.

Other fluxes often become useless at the 20 end of a single day through vaporization or the accumulation of oxids, making the flux very heavy, or causing it to stick to the articles when immersed. The compound flux spreads freely upon the molten bath, and 25 protects it so effectively from oxidation that the flux does not become clogged with oxids.

From the above description it will be seen that the advantages of using zinc chlorid are attained without the liability to vaporization of the same, and at an expense enormously less than a flux of zinc chlorid would cost.

In H. J. Lohmann's Patent No. 990,443 granted April 25, 1911 for process of combining a permeating metallic protective with the surface of ferric articles, a treatment of iron and steel articles with a salt of mercury is described, to render the surface of the article more receptive of lead, zinc and 40 tin alloys; and it is found that the use of the flux claimed herein is especially advantageous in the coating of such articles in a molten bath, as it prevents the oxidation of the mercury and serves to clean any oxidized 45 spots upon the surface of the article, so that a perfect coating may be formed thereon. The process of depositing the salt of mercury upon such articles is fully set forth in the said Patent No. 990,443, and does not 50 need to be described herein, as it forms no part of the present invention.

The efficiency of the flux in every respect is very great, and the advantage due to its cheapness is evident from the foregoing 55 considerations.

When the flux is prepared upon the surface of the molten metal in the manner described above, the zinc chlorid forms less than one-fourth of the entire flux, but operates as efficiently as a flux formed chiefly 60 of zinc chlorid.

### Claims:

1. The process of forming a flux upon a bath of fusible metal as lead, zinc and tin, which consists in applying a solution of zinc 65 chlorid to the surface of the molten metal insufficient to cover its surface and adding ammonium chlorid thereto until the mixture covers the surface of the bath.

2. The process of forming a flux upon a 70 bath of fusible metal as lead, zinc and tin, which consists in applying a solution of zinc chlorid saturated with ammonium chlorid to the surface of the bath insufficient to cover its surface, and adding ammonium chlorid 75 thereto until the mixture covers the surface of the bath.

3. The process of applying a metal coating to ferrous articles, which consists in coating the surface of the metal bath with a 80 flux of zinc chlorid and ammonium chlorid, then depositing a salt of mercury upon the surface of the ferrous article, and finally passing such article with such salt of mercury through the flux into the molten bath. 85

4. The process of applying a coating chiefly of lead, to ferrous articles, which consists in coating the surface of a molten lead bath with a flux of zinc chlorid and ammonium chlorid, then depositing a salt of 90 mercury upon the surface of the ferrous articles, and finally passing the article thus treated through the flux into the bath of melted lead.

5. The process of applying a metal coating to ferrous articles, which consists in coating the surface of the metal bath with a flux of zinc chlorid and a considerable excess of ammonium chlorid, then immersing the 95 ferrous article in a liquor of cleaning acid 100 mixed with a salt of mercury, and finally passing the article through the melted flux into the molten metal.

6. The process of forming a flux upon a bath of fusible metal, as lead, zinc, and tin, 105 which consists first, in applying zinc chlorid to the surface of the metal in quantity insufficient to cover the said surface, second, evaporating such zinc chlorid until it coheres in a mass, and third, adding ammonium chlorid sufficient to form a thick liquid 110 covering the surface of the metal to a depth of not less than one-eighth of an inch.

In testimony whereof we have hereunto set our hands in the presence of two sub- 115 scribing witnesses.

JAMES H. MADDY.  
BRUNO H. SCHUBERT.

Witnesses:

J. G. BELDEN,  
A. J. RAY.